

April 22, 1924.

1,491,280

P. C. WENTWORTH

RING TRAVELER

Filed May 19, 1923

FIG.1



FIG.2



FIG.3



FIG.4



FIG.5



FIG.6



Inventor  
Philip C. Wentworth  
Assignee  
S. S. Speary & Co.  
By Attorney

Patented Apr. 22, 1924.

1,491,280

# UNITED STATES PATENT OFFICE.

PHILIP C. WENTWORTH, OF PROVIDENCE, RHODE ISLAND.

## RING TRAVELER.

Application filed May 19, 1923. Serial No. 640,251.

To all whom it may concern:

Be it known that I, PHILIP C. WENTWORTH, a citizen of the United States, residing at Providence, county of Providence, State of Rhode Island, have invented certain new and useful Improvements in Ring Travelers, of which the following is a specification.

My present invention relates to ring travelers and particularly to a hardened and tempered traveler in which there is great hardness at the horns and a resiliency or spring temper in the bows.

In my previous application Patent No. 1,461,059, the traveler therein described as an illustrative embodiment and the method of producing it dealt more particularly with travelers in which the amount of carbon was uniform or substantially uniform throughout, but the amount of converted carbon varied. In accordance with my present invention I contemplate a traveler in which a differential or variant temper or hardness is secured and in this class the traveler has a difference between horns and bow in the amount of carbon in these respective parts. In this form of my invention there may or may not be a difference in the proportion between the hardening carbon and the cement carbon.

As illustrative of my invention I shall describe a traveler in accordance with my invention and indicate briefly the method of effecting this variable carbonization. In the drawings forming a part hereof I am of necessity obliged to resort to somewhat diagrammatic treatment. In these drawings:—

Fig. 1 is a somewhat diagrammatic section through a traveler in accordance with my invention.

Figs. 2 to 5 are similar views showing successive stages in the method of hardening such a traveler, and

Fig. 6 is a diagrammatic indication of a mechanical handling of the process.

My new traveler as heretofore suggested has for its principal characteristic a variation of carbon content between the horns H and the bow B. This I have endeavored to illustrate diagrammatically in Fig. 1 in which the traveler T may be considered as illustrated in diagrammatic section to expose or make visible the aforementioned variation in the carbon content of its metal. The variations in heaviness of the section lines are intended to represent variations in

percentage of carbon in the metal of the traveler and not as in my prior Patent No. 1,461,059, a variation in the proportion of the dissolved or hardening carbon. Again and to make this clear, in my said patent I was dealing with a traveler of substantial uniform carbon content throughout but variably tempered so that the percentage of dissolved or hardening carbon to the cement carbon varied. In my present case the actual amount of carbon in the metal varies from the horns H up to the bow B. There may or may not be any variation in percentage of cement and hardening carbon as that is more or less immaterial in accordance with my present invention.

The traveler herein involved while having a similar characteristic hardness at the horns and spring temper at the bow is distinguished by its actual variation of carbon content which is the principle involved in my present invention.

While my variant carbon traveler may be variously treated for production I have shown in Fig. 6 as a diagrammatic indication of the handling of the process a shallow tank 1 in which a molten bath 2 of any suitable carbonizing material such as a fusible carbonaceous compound, a cyanide, ferrocyanide or carbonate, either sodium or potassium. In this form the bath 2 is kept molten by the burners 3. The formed but uncarbonized travelers T<sup>1</sup> which may be considered as made from stock of uniform very low carbon content are fed onto a wire guideway such as 4 by any suitable form of feeding device such as is ordinarily used to pick up and drop articles of this class. This guideway 4 inclines gradually downward until it reaches the surface of the molten bath 2 from which it begins to rise again until it reaches a downward turn or loop 4<sup>1</sup> disposed over a quenching tank 5. The travelers T<sup>1</sup> are picked up one by one by fingers 6 of a chain or belt 7 running over pulleys 8. The chain or belt 7 is given sufficient slack to permit it to follow in substantial parallelism with the course of the guideway 4. The travelers are thus slowly propelled through the bath by a gradual submersion and emersion until they come out over the end 4<sup>1</sup> where they automatically drop off.

I have endeavored to indicate by exponents for the character T that the uncarbonized traveler T<sup>1</sup> as indicated in Fig. 2 move down to the surface of the liquid and when they

begin to enter that surface take on carbon at their horns as indicated at T<sup>2</sup>, Fig. 3. As they are advanced they reach a great depth as at T<sup>3</sup> in Fig. 4 and gradually having been 5 submerged at the central area of the tank emerge finally as T as indicated in Fig. 5 which corresponds to the state in Fig. 1.

Various modifications may be made in the 10 method of progressively treating the travelers with the carbon yielding medium whether it be molten or otherwise and the mechanical handling may be variously effected. Various 15 modifications thus made in accordance with the spirit of my invention are to be considered as included thereby if within the limits of the appended claims.

What I therefore claim and desire to secure by Letters Patent is:

1. A hardened ring traveler of the class described comprising a bow and terminal horns 20 and having more carbon per unit of cross section at the horns than at the bow.

2. A hardened ring traveler of the class described comprising a bow and terminal 25 horns formed of low carbon metal and carbonized so as to have more carbon per unit of cross section at the horns than at the bow.

3. A ring traveler of the class described 30 comprising a traveler formed of low carbon metal and having a decreasing amount of carbon per unit of cross section from the horns towards the bow.

4. The method of making a hardened ring 35 traveler consisting in forming a traveler

from stock of uniform low carbon content, and in treating the traveler so formed to introduce therein more carbon per unit of cross section at the horns than at the bow.

5. The method of making a hardened ring 40 traveler consisting in forming a traveler from stock of uniform low carbon content, and in treating the traveler so formed to introduce therein progressively decreasing amounts of carbon per unit of cross section 45 from the horns towards the bow.

6. That step in the method of making a hardened ring traveler which consists in introducing into a piece of stock of uniform low carbon content more carbon per unit of 50 cross section at the horns than at the bow.

7. That step in the method of making a hardened ring traveler which consists in introducing into a piece of stock of uniform low carbon content progressively decreasing 55 amounts of carbon per unit of cross section from the horns towards the bow.

8. That step in the method of making a hardened ring traveler which consists in introducing into a piece of stock of uniform 60 low carbon content more carbon per unit of cross section at the horns than at the bow and in amounts progressively decreasing from the horns towards the bow.

In testimony whereof I affix my signature 65 in presence of two witnesses.

PHILIP C. WENTWORTH.

Witnesses:

N. C. THOMAS,  
E. B. ALLEN.